

(No Model.)

3 Sheets—Sheet 1.

O. S. GARRETSON.

## METHOD OF AND APPARATUS FOR BESSEMERIZING MATTE.

No. 596,992.

Patented Jan. 11, 1898.



**WITNESSES:**

Chas. F. Burkhardt,  
Ernest Pufendorf.

*O. S. Garrison*

By William Rownd

**INVENTOR.**

**ATTORNEYS.**

(No Model.)

3 Sheets—Sheet 2.

O. S. GARRETSON.

METHOD OF AND APPARATUS FOR BESSEMERIZING MATTE.

No. 596,992.

Patented Jan. 11, 1898.



WITNESSES:

Chas. F. Burkhardt,

Emes & Pulford.

O. S. Garretson

INVENTOR.

By Wilhelm Sommer.

ATTORNEYS.

(No Model.)

3 Sheets—Sheet 3.

O. S. GARRETSON.

## METHOD OF AND APPARATUS FOR BESSEMERIZING MATTE.

No. 596,992.

Patented Jan. 11, 1898.



*Witnesses*

Chas. F. Burkhardt  
Henry L. Deck

O.S. Garrelson Inventor.

By William Storner.  
Attorneys.

# UNITED STATES PATENT OFFICE.

OLIVER S. GARRETSON, OF BUFFALO, NEW YORK.

## METHOD OF AND APPARATUS FOR BESSEMERIZING MATTE.

SPECIFICATION forming part of Letters Patent No. 596,992, dated January 11, 1898.

Application filed November 13, 1896. Serial No. 811,997. (No model.)

To all whom it may concern:

Be it known that I, OLIVER S. GARRETSON, a citizen of the United States, residing at Buffalo, in the county of Erie and State of New York, have invented new and useful Improvements in Methods of and Apparatus for Bessemerizing Matte, of which the following is a specification.

This invention has reference to the treatment of matte by the converting or bessemerizing process. This process is now generally carried on in converting vessels which are provided with a silicious lining, which furnishes the silica for the combination with the iron oxid produced by the action of the blast upon the iron contained in the matte. The matte is treated in these converters in a charge at a time, and the lining is eaten away by each charge to a certain extent, so that the lining is required to be renewed after a certain number of charges have been treated. The operation of these converters is intermittent. The slag is poured off by tipping the converter when the proper stage has been reached, and the finished charge is finally poured out. The converter is then ready to receive another charge unless the lining has been eaten out to such an extent that the converter requires to be relined. The converter is then relined and dried, which operations consume considerable time and labor.

My invention has for one of its objects to convert or bessemerize the matte by a continuous operation, in which the silicious matter is supplied to the converter from time to time, as may be necessary to maintain the proper amount of silicious matter in the converter, and in which the matte is supplied to the converter continuously, or nearly so, so that fuel, consisting of the oxidizable ingredients contained in raw matte, is continuously supplied to the charge in the converter.

My invention has for a further object the separation of different metals contained in complex ore or mattes by converting or bessemerizing the matte successively in different communicating chambers or compartments, whereby the metallic constituents of the ore or matte which are most readily precipitated are separated and deposited first, and other less readily-precipitated metals are separated

and deposited in the following compartment or compartments.

In the accompanying drawings, consisting of three sheets, Figure 1 is a longitudinal vertical section of a smelting-furnace which is provided with two communicating converting-furnaces according to my invention. Fig. 2 is a horizontal section in line 2 2, Fig. 1. Fig. 3 is a vertical section of a detached converting-furnace by which my improved method of converting or bessemerizing can be practiced. Fig. 4 is a horizontal section in line 4 4, Fig. 3. Fig. 5 is a fragmentary cross-section of the top of the furnace at right angles to Fig. 1 on an enlarged scale. Fig. 6 is a sectional elevation, on an enlarged scale, of one of the gas-escape valves.

Like letters of reference refer to like parts in the several figures.

A represents a smelting or main furnace, which has a slag-outlet *a* at one end or side and a matte-outlet *b* at the opposite end or side and which is preferably long and narrow. The bottom *c* of the furnace is preferably slightly sloped from the slag-outlet toward the matte-outlet, so that the flow of the heavier ingredients of the molten material is directed toward the matte-outlet. The lower edge of the matte-outlet is preferably arranged on a slightly lower level than the lower edge of the slag-outlet.

*d* represents the tap-hole, through which the metal or metallic compounds can be withdrawn from the bottom of the furnace when desired.

*E* represents the tuyers of the furnace, by which a blast suitable for smelting is supplied to the furnace and which are arranged above the slag-level in a common manner. The blast which is supplied to these tuyers is preferably heated by any suitable heating apparatus, but I prefer for that purpose the hot-blast apparatus which forms the subject-matter of my application for Letters Patent filed October 29, 1896, Serial No. 610,403. In this hot-blast apparatus the blast is heated by the discharged molten slag in a conduit *F*, through which the slag is conducted by an endless carrier *g*. The blast passes from this conduit through two conduits *G'*, which are arranged on opposite sides of the furnace.

and from which the twyers are supplied in a well-known manner. The conduits  $G'$  are provided with valves  $g'$  for regulating or shutting off the blast and with suitable hand-holes  $G^2$ .

The top portion of the furnace is constructed in any suitable or well-known manner—for instance, with pivoted doors  $G^3$ , Fig. 5, for feeding the ore and flux to the furnace and permitting the escape of the gases through the uptakes  $II$ .

I represents the forehearth or settling-well, which receives the slag from the slag-outlet  $a$  of the furnace and which may be constructed in any suitable manner. I prefer, however, a forehearth constructed as described and claimed in my application for Letters Patent filed November 7, 1896, Serial No. 611,338. In this forehearth the bottom  $i$  is arranged practically on a level with the bottom of the slag-outlet  $a$  of the furnace or slopes slightly toward said outlet, so that matte or other molten metallic compounds which may settle to the bottom of the forehearth flow back into the furnace.

$i'$  is the slag-outlet of the forehearth, which outlet is arranged higher than the slag-level of the furnace. The air-pressure in the furnace drives the slag to the outlet of the forehearth, from which it passes to the slag-inlet  $j$  of the hot-blast apparatus. This pressure is maintained in the furnace, as is well known, because the stack of the furnace is filled with a column of ore and fuel, through which the blast must force its way in order to escape. If necessary, the forehearth may be kept filled with charcoal, through which the slag is filtered before escaping and whereby any further values contained in the slag are filtered out or reduced. The forehearth may be provided with twyers  $J$  for supplying air to burn a part of the charcoal sufficient to maintain the heat which is necessary to keep the slag sufficiently fluid.

K represents the pipe through which the gases escape from the forehearth and which is preferably connected with the forehearth immediately above its slag-outlet.

L represents the bell or cover in the feed-hopper  $l$  of the forehearth.

M represents an upright converting-furnace or bessemerizing apparatus which is arranged adjacent to the matte-outlet  $b$  of the furnace and receives the matte therefrom. M' represents a second converting-furnace arranged adjacent to the first converting-furnace M and receiving the matte therefrom. Each of these converting-furnaces has its body composed of an upright water-jacketed column, stack, or shell  $m$  of cylindrical, prismatic, or other suitable form, and has a depressed bottom  $m'$ , provided with a suitable tap-hole  $m^2$ . The first converting-furnace M is provided in the side of its shell with an opening  $o$ , which coincides with the matte-outlet  $b$  of the furnace, and on its opposite side with an opening  $o'$ , which coincides with

the opening  $h$  of the second converting-furnace M'. The openings  $h o o'$  are made of sufficient area to permit of the free escape of the gases from the converting-furnaces to the main furnace. Each of the converting-furnaces may, however, be provided with a supplemental gas-escape passage  $P$ , which leads to the uptake of the main furnace and which is closed by a weighted valve  $p$  of any suitable construction, (indicated by dotted lines in Fig. 1,) so that the gases can escape through this supplemental passage upon forcing said valve open should their escape to and through the main furnace be obstructed. Each of these converting-furnaces is provided with twyers  $q$ , through which a blast suitable for converting or bessemerizing the matte is injected into the molten matte. These twyers are arranged at such a height above the bottom of the furnace that they deliver the blast into the zone occupied by the molten matte, which zone lies above the zone occupied by the metal on the bottom of the converting-furnace and below the slag-level. The blast which is supplied to these twyers need not be heated and can be conducted to the twyers by flexible pipes  $q'$ . Each of these converting-furnaces may also be provided above the slag-level with twyers  $q^2$ , through which an additional air-supply may be injected, if necessary. The converting-blast is injected under a sufficiently high pressure to enable the blast to penetrate the molten matte, which pressure may range from four to five pounds or more per square inch, while the smelting-blast is injected at a much lower pressure, which may range from one-half to one and one-half pounds.

The bottom of each converting-furnace is arranged so far below the matte-inlet opening  $o$  in the side of the furnace that the molten metal or metallic compound which collects on the bottom of the converting-furnace will remain there and will not flow back to the main furnace or pass on to the next converting-furnace.

S represents the top plate of each converting-furnace, which is provided with a feed-hopper  $s$ , closed by a bell or valve  $s'$ .

The converting-furnaces may be supported on wheels  $t$ , as shown, so that each can be removed and replaced by another furnace, if necessary, or they may be stationary, as may be preferred.

In practicing my invention a matte is produced in the smelting or main furnace A in any suitable manner—for instance, by smelting sulfid ores in the presence of a suitable flux, such as quartz, diorite, &c. The matte accumulates on the bottom of the smelting-furnace and flows slowly toward the first converting-furnace and enters the same and passes from the first to the second converting-furnace. The matte may become so concentrated in the smelting-furnace that the metals which are most easily precipitated, such as bismuth and lead, separate themselves from

the matte and collect on the bottom of the smelting furnace. The metal which is there deposited is drawn off from time to time through the tap-hole d. The bulk of the matte 5 enters the first converting-furnace M and is subjected in the same to the converting-blast, whereby the combustible ingredients—such as sulfur, iron, arsenic, &c.—are to a large extent burned out. The converting-furnaces 10 are filled with a column of flux in lumps—such as quartz, diorite, or other mineral containing a large percentage of silica. The weight of this column keeps the lower portion 15 of the same pressed down into the layer of matte, so that the iron oxid which is being formed in the matte by the oxidizing-blast can come in contact with the silica and combine with the same to a silicate, which forms a liquid slag. The latter rises to the surface of 20 the molten material and flows back into the main furnace through the openings o b and joins the slag produced in the main furnace. The matte which is treated in the first converting-furnace becomes richer as the treatment proceeds and deposits the metal which 25 is reduced to the metallic state and which may contain considerable copper if the bulk of the bismuth and lead has been precipitated in the main furnace. If no metal has been precipitated in the main furnace, the first converting 30 operation will cause the precipitation of lead and bismuth principally, if the matte contains these metals. The matte is further subjected to the action of a converting-blast in 35 the second converting-furnace, and the metal which is precipitated in the second converting-furnace consists largely of copper. If the ore which is being smelted in the main furnace is very complex, a third converting-furnace 40 may be employed. When the matte flows successively through several of these converting-furnaces, the metals contained in the matte are separated to a greater or less extent and precipitated in the several furnaces as alloys in which one or the other metal 45 predominates. The slag which is formed in the second converting-furnace flows back to the first furnace and thence into the main furnace. The slags formed in the converting-furnaces are comparatively rich and are compelled 50 to pass through the main furnace before they can reach the forehearth or final slag-outlet. In passing through the main furnace these slags encounter the sulfur which is there in excess and the poor matte which 55 is rich in sulfur. The sulfur combines with the metal and oxidized carried by the slag and forms therewith matte, which joins the matte being formed and returns with the same to the converting-furnaces. In this manner a 60 flow of matte is kept up through the main furnace toward and through the converting-furnaces and of slag from the converting-furnaces to and through the main furnace. The 65 slag which enters the forehearth parts in the latter with any values which it may still con-

tain and which return to the main furnace, while the slag is finally discharged in a practically clean state. The metal which is precipitated in the main furnace and in the converting-furnaces is drawn off from time to time through the tap-holes.

In the above-described method of conversion or bessemerizing the converting-chamber is constantly supplied with fresh matte, 75 and as the latter carries in its constituents a sufficient amount of oxidizable substances, such as sulfur and iron, to serve as fuel in the converting or bessemerizing operation the latter can be continued indefinitely without 80 danger of chilling for want of fuel. The supply of flux or silica is also constant, or nearly so, as the column of flux in each converting-furnace is replenished at the top from time to time, as may be required, so that the silica is 85 always abundantly present for combination with the iron oxid which is being formed. A water-jacketed furnace can therefore be used in this converting process, as indicated in the drawings, because no silicious lining is 90 required for furnishing the silica necessary for forming slag, as in an ordinary converter.

As the converting process is continuous and the slag flows off continuously, a large amount of time and labor is saved, no handling being 95 required for supplying the matte or returning the slag to the main furnace for treatment, it being only necessary to maintain the supply of ore and flux and to remove the finished product from time to time.

In some cases it may not be desirable to carry the process of conversion to the extent that metal is actually precipitated, but only far enough to concentrate or enrich the matte preparatory to further treatment. This depends largely upon the nature of the ores and upon local and other conditions and can be readily accomplished, when desired, by properly regulating the converting operation.

My improved converting or bessemerizing method can also be practiced without returning the slag to the smelting or main furnace. In Fig. 3 is represented a converting or bessemerizing furnace M<sup>2</sup>, which is in all material respects constructed like the converting-furnaces M M' hereinbefore described, but which is not directly connected with a smelting-furnace. This converting-furnace is supplied with molten matte through a spout u either continuously or from time to time, as 110 may be most convenient, and the liquid slag escapes through an outlet u' either continuously or from time to time. The furnace is kept charged with a column of silicious material, as hereinbefore described, which material is supplied through a door u<sup>2</sup> in the upper portion of the furnace, and the gases escape through a pipe u<sup>3</sup>. The slag which is discharged from this furnace must be treated 115 separately if it is sufficiently rich to warrant such treatment. If necessary, a small amount of carbonaceous fuel may be supplied to this

furnace with the flux. If desired, the matte may be supplied to this furnace in lumps or pigs instead of in a molten condition.

I claim as my invention—

- 5 1. The herein-described method of converting or bessemerizing matte which consists in subjecting the molten matte to a converting or bessemerizing blast underneath a column of flux or silicious material, substantially as set forth.
- 10 2. The herein-described method of converting or bessemerizing matte which consists in supplying the molten matte continuously to a converting or bessemerizing chamber and subjecting the matte to a converting or bessemerizing blast therein underneath a column of flux or silicious material, substantially as set forth.
- 15 3. The herein-described method of converting or bessemerizing matte which consists in supplying the molten matte continuously to a converting or bessemerizing chamber, subjecting the matte therein to a converting or bessemerizing blast underneath a column of flux or silicious material, and removing the slag continuously from said chamber, substantially as set forth.
- 20 4. The herein-described method of smelting and converting or bessemerizing matte which consists in smelting the ore to produce matte, causing the matte to flow continuously from the smelting-chamber to a separate converting or bessemerizing chamber, subjecting the matte in the latter to a converting or bessemerizing blast underneath a column of flux or silicious material, and causing the slag to flow from said converting or bessemerizing chamber to said smelting-chamber, substantially as set forth.
- 25 5. The herein-described method of separating the metallic constituents contained in complex ores or mattes which consists in smelting the ore to produce matte, causing the matte to flow from the smelting-furnace into several successive converting or bessemerizing furnaces, subjecting the matte to converting or bessemerizing blasts in the lat-

ter and forming a fluid slag therein, causing such slag to flow from said converting or bessemerizing furnaces to said smelting-furnace where the slag is acted upon by the sulfur and sulfids before it is discharged from the smelting-furnace, and withdrawing the deposited metallic constituents separately from said converting or bessemerizing furnaces, substantially as set forth.

6. The combination with a smelting-furnace, of a separate converting or bessemerizing furnace having air-ports or twyers and having a stack adapted to hold flux, said converting-furnace communicating with the smelting-furnace by a passage which is arranged in the lower portions of the adjacent side walls of said furnaces and adapted to allow the matte to flow from the smelting-furnace into the converting-furnace and the slag to flow from the converting-furnace into the smelting-furnace, substantially as set forth.

7. The combination with a smelting-furnace, of a separate converting or bessemerizing furnace having air-ports or twyers and having a stack adapted to hold flux, said converting-furnace communicating with said smelting-furnace by a passage which is arranged in the lower portions of the adjacent side walls of said furnaces and adapted to allow the matte to flow from the smelting-furnace into the converting-furnace and the slag to flow from the converting-furnace into the smelting-furnace and a forehearth arranged at the opposite side of the smelting-furnace and receiving the slag therefrom, whereby the slag formed in the converting-furnace is compelled to flow through the smelting-furnace and is subjected to the action of the sulfur and sulfids therein in passing to the forehearth, substantially as set forth.

Witness my hand this 10th day of November, 1896.

OLIVER S. GARRETSON.

Witnesses.

JNO. J. BONNER,  
E. R. DEAN.